

# UNITED STATES PATENT OFFICE.

ERNEST WYNDHAM MERRY, OF SHEFFIELD, ENGLAND, ASSIGNOR TO INTERNATIONAL PYROTAN COMPANY, LIMITED, OF LONDON, ENGLAND.

## TANNING OF HIDES AND SKINS.

1,191,527.

Specification of Letters Patent. Patented July 18, 1916.

No Drawing.

Application filed January 12, 1916. Serial No. 71,652.

*To all whom it may concern:*

Be it known that I, ERNEST WYNDHAM MERRY, subject of the King of Great Britain and Ireland, residing at 45 Cherry street,

5 Bramall Lane, Sheffield, in the county of York, England, have invented new and useful Improvements in the Tanning of Hides and Skins, of which the following is a specification.

10 This invention relates to the tanning of hides and skins by the action of the known mineral agents, alum and pyrophosphate of sodium and has for its object the carrying out of the tanning operation with hides or 15 skins of any character or thickness with thoroughness and certainty in a simple and controllable manner.

I am aware that a process has been described in the specification of the United 20 States Patent No. 1,039,150 in which the agents above referred to have been included in the ingredients of a tanning solution or 25 solutions of definite strength which it is therein stated may be varied to suit the different classes and weights of hides being 30 treated and specific proportions of the several ingredients are given as being effective for cow hides of a medium weight. I have discovered that the said process, however, 35 is only applicable to cow hides and other similar hides of a loose character and small thickness and that when thick hides or hides of a firm character such as ox hides are under treatment it is impossible to produce 40 a satisfactory tannage even by increasing the strength of the tanning solution by 50%.

As the result of numerous experiments I believe that the permanent tanning action of 45 a solution containing alum and sodium pyrophosphate is due to the interaction in the pores of the hide of the alum and the sodium pyrophosphate, whereby there results pyrophosphate of aluminium, which latter is insoluble in water and becomes fixed 50 in the pores of the hide.

My present invention consists in the provision of a tanning solution or solutions of such composition and concentration as are 55 hereinafter set forth and within the limits defined. By observing these limits the tan-

ning operation can be effected on any class or thickness of hide with a celerity, certainty and efficiency which is not at present attainable by known means.

In describing how my present invention 55 is carried into effect I shall define the proportions employed as a percentage of the weight of hide to be treated. Sodium pyrophosphate as it is found in commerce contains a varying quantity of the pure anhydrous salt, say, from 45 to 65 per cent. thereof, therefore in the percentages herein-after given it must be understood that the same are based on the pure anhydrous salt 60  $Na_4P_2O_7$ .

According to my present invention; the alum (I refer to the crystallized salt with 24 molecules of water of crystallization) must exceed 5 and should not exceed 7 times the weight of sodium pyrophosphate, for example 10% of the former and 1.66% of the latter and the water must be between 20% and 40% of the weight of hide treated, for example 27%. While this latter concentration gives the greater penetrating effect any 75 much higher concentration than this is not desirable owing to the risk of graining taking place due to the solution being too small in volume to permit of the uniformity of strength being maintained throughout the 80 whole of the volume of solution, particularly that portion between the layers of hide.

The composition of the tanning bath is as follows: 10% ammonia alum,  $(NH_4)_2SO_4Al_2(SO_4)_324H_2O$ ; 1.66% pyrophosphate of soda,  $Na_4P_2O_7$ ; 27% water, and say 5% of common salt, or its substitute.

The preliminary treatment of soaking and liming of the hides is carried out by any of 90 the common methods; the limed hides being subsequently surface delimed with boracic acid in the well known way. They are then drummed in a solution of borax in water or boracic acid in water at an initial temperature of from 90°-100° F. for 10 minutes. The solution is then drained off and a fresh quantity introduced into the drum. After a further 10 minutes drumming the solution 95 is again drained away and the hides finally 100

washed in the drum with warm water at 80°-90° F. The hides are then subjected to the action of a tanning bath containing alum, common salt or some similar substance 5 to counteract the drawing effect of the alum, and sodium pyrophosphate in water at an initial temperature of 80°-90° F. until the hide is completely penetrated. This bath is preferably prepared by dissolving the alum, 10 and common salt or its substitute in the desired quantity of hot water and dissolving the sodium pyrophosphate in a separate quantity of hot water and mixing the two solutions together. An alternative method 15 which produces the same result is to thoroughly mix the substances mentioned in the dry state and dissolve this mixture in the requisite amount of hot water. The tanning bath however prepared is then placed in the 20 drum with the hides and drummed for 45 minutes or the tanning bath may be added by degrees to the drum if so desired. The mixture after drumming is then run off into another vessel and the hides transferred to 25 such vessel and placed in the mixture therein or what is usually more convenient the hides and mixture are left in the drum, care being taken that no creasing or marking occurs. The tanning is allowed to progress for 3-4 30 hours or longer until the hides are tanned through. Alternate drumming and resting may be used to accelerate the process if close heavy hides are being treated. The tanned hides are then horsed up for 12 hours 35 (usually overnight). The liquor in the drum is then mixed with the coloring bath which may be added direct to the drum. The coloring bath is obtained by dissolving each of the desired materials usually 40 gambier and quebracho, in separate quantities of hot water and finally mixing the solutions obtained in the usual manner. 3% gambier and 2% quebracho dissolved in as small a quantity of water as possible will be 45 found suitable but these quantities may be varied. The hides are rapidly replaced and drummed for 3 hours. A rather safer method is to drum the hides in the exhausted tanning bath liquor and then gradually add 50 the prepared coloring bath during that process through the axle of the drum in well known manner.

For certain classes of leather such as sole leather and for close heavy hides it is sometimes found advisable to supplement the tanning process by the following treatment:—Taking the hides out of the tanning bath and giving them a supplementary bath which is added in two stages prior to the coloring bath. The first stage consists in the addition of a supplementary bath to the exhausted tanning bath liquor contained in the drum. The hides are then inserted and drummed for 45 minutes. The supplementary bath is prepared in a similar manner

to the tanning bath described above. Its composition is:—5% ammonia alum, 1.66% pyrophosphate of soda, 27% water, and say 5% common salt or its substitute.

The second stage consists in the further 70 addition to the mixture in the drum of a solution of alum dissolved in as little hot water as possible; the quantity of alum being the same as that used in the supplementary bath. Drumming is now continued for 75 a further 2 hours and the whole then allowed to stand 12-14 hours after adjusting the hides in the drum to prevent creasing. The hides are then colored by the addition of the coloring bath to the mixture in the drum 80 using the same method as already described. The resulting colored hides whether prepared by the single or double bath process are finally horsed up for 12-14 hours and then rinsed through a bath which may consist of water alone or a ½% solution of borax. After draining, the hides are then finished by one of the well known processes 85 in the usual way.

I would have it clearly understood that 90 any soluble aluminium salt may be substituted for the ammonia alum herein referred to such for example as soda alum  $Na_2SO_4Al_2(SO_4)_3 \cdot 24H_2O$ , potash alum  $K_2SO_4Al_2(SO_4)_3 \cdot 24H_2O$ , or aluminium sulfate  $Al_2(SO_4)_3 \cdot 18H_2O$ . 95

In using these salts the relative proportions in the formulæ given must be modified so as to maintain the aluminium constituent at its proper value.

I claim:—

1. In a process of tanning by means of alum and sodium pyrophosphate the treatment of the hides in a tanning solution in which the proportion of alum in terms of 105 the crystallized salt with 24 molecules of water of crystallization to sodium pyrophosphate in terms of the pure anhydrous salt is in the ratio exceeding 5 up to 7 parts of alum to 1 part of sodium pyrophosphate. 110

2. In a process of tanning by means of alum and sodium pyrophosphate the treatment of the hides in a tanning solution in which the proportion of alum in terms of 115 the crystallized salt with 24 molecules of water of crystallization to sodium pyrophosphate in terms of the pure anhydrous salt is in the ratio exceeding 5 up to 7 parts of alum to 1 part of sodium pyrophosphate the proportion of the said alum being substantially  $\frac{1}{10}$ th of the weight of hide treated. 120

3. In a process of tanning by means of alum and sodium pyrophosphate the treatment of the hides in a tanning solution in which the proportion of alum in terms of 125 the crystallized salt with 24 molecules of water 27%, alum 10%, sodium pyrophosphate in terms of the pure anhydrous salt is in the ratio exceeding 5 up to 7 parts of alum to 1 part of sodium pyrophosphate the 130

restriction of the quantity of the water in the tanning bath to from 20% to 40% of the weight of hide treated.

4. A tanning solution of the following proportions on the weight of hide treated, water 27%, alum 10%, sodium pyrophosphate 1.66% and, say, 5% of a pore opening agent such as common salt.

In testimony whereof I have signed my name to this specification in the presence of 10 two subscribing witnesses.

ERNEST WYNDHAM MERRY.

Witnesses:

DORIS H. HITCHCOCK,  
CHARLES J. R. BULLOUGH.